

## UNITED STATES PATENT OFFICE

RICHARD ELSSNER, OF JOHNSON CITY, TENNESSEE, ASSIGNOR TO AMERICAN GLANZ-  
STOFF CORPORATION, OF NEW YORK, N. Y., A CORPORATION OF DELAWARE

## EVENNESS OF SHRINKAGE

No Drawing.

Application filed August 29, 1931. Serial No. 560,225.

My present invention concerns a new method of wet-treating artificial filaments i. e. filaments formed synthetically, specifically from cellulosic solutions.

5 One object of my invention is to so wet-treat filaments that an even shrinkage results.

For matter of convenience the present application is described with respect to the 10 viscose process, but it must be understood that my new invention may be used in any process where spun filaments must be wet-treated.

15 In the manufacture of filaments, and films, from a viscose solution, the extruded product is usually passed through an acid bath in order that it may be hardened, or precipitated. In the case of artificial viscose filaments, for example, the product is usually 20 wound upon foraminated or perforated spools or bobbins. The filaments must then be deacidified, desulphurized, and washed. When drying these yarns upon the perforated spools an uneven drying and shrinkage of 25 the filaments usually results. This causes unevenness in the quality of the yarn produced, and affects the dyeing properties.

According to my new process, a series of 30 dryings is accomplished, and thus an evenness of shrinkage results.

My process, with respect particularly to viscose yarns, for example, is as follows:

The yarn, wound upon a foraminated spool 35 is wet-treated in the usual way, and then dried. The yarn body is then re-wet, and dried. Then the filaments are rewound or twisted, onto another similar spool, in such a manner that a loose yarn body is obtained; and again wet and dried. Then a fourth 40 wetting and drying is performed and the resulting filaments have been found to possess a technically even shrinkage and the corresponding desirable dyeing properties.

The drying may be accomplished in any 45 well-known manner, and I do not wish to have my present invention limited to any type of drying. I wish to have my invention limited only by the scope of the appended claims.

50 The wetting may be accomplished by

spraying with water or aqueous solutions, or by dipping in water or aqueous solutions.

I claim:

1. In a process for treating wet artificial filaments wound upon a spool or bobbin, the 55 steps of drying, rewetting and redrying the filaments, rewinding onto another spool or bobbin, rewetting, redrying, rewetting and redrying the filaments.

2. In a process for obtaining an evenness 60 of shrinkage of spun filaments, the steps of winding the same on a spool or bobbin, wet-treating and drying, rewetting and redrying the same, rewinding onto another similar spool or bobbin, and repeating the wetting and drying a plurality of times.

3. In a process for obtaining an evenness 65 of shrinkage of spun filaments, the steps of winding the same on a spool or bobbin, wet-treating and drying, rewetting and redrying the same, rewinding and twisting onto another similar spool, and repeating the wetting and drying until altogether four dryings have been performed.

4. In a process for obtaining an evenness 75 of shrinkage of spun filaments, the steps of winding the same on a spool or bobbin, wet-treating, and drying, rewetting and redrying the same, rewinding onto another similar spool, and repeating the wetting and drying a plurality of times while thereon.

In testimony whereof I affix my signature.

DR. RICHARD ELSSNER.

85

90

95

100